

Oct. 9, 1951

H. A. ROBINSON ET AL.  
SACRIFICIAL ANODE SYSTEM FOR PROTECTING  
METALS IN SEA WATER  
Filed June 15, 1949

2,571,062



Fig. 2



Fig. 4



Fig. 1



Fig. 5



Fig. 3

INVENTORS.  
Harold A. Robinson  
Hilary A. Humble

BY  
Griswold & Burdick  
ATTORNEYS

## UNITED STATES PATENT OFFICE

2,571,062

## SACRIFICIAL ANODE SYSTEM FOR PROTECTING METALS IN SEA WATER

Harold A. Robinson and Hilary A. Humble, Midland, Mich., assignors to The Dow Chemical Company, Midland, Mich., a corporation of Delaware

Application June 15, 1949, Serial No. 99,156

4 Claims. (Cl. 204—197)

1

This invention relates to a sacrificial anode system for protecting corrodible metal structures immersed in seawater.

The tendency for structures of steel and similar metals, when immersed in seawater, to undergo serious corrosion can be offset by cathodic protection. In this process the structure is made the cathode in an electric circuit using the seawater as electrolyte. If sufficient current is supplied, the structure can be kept from corroding.

Such cathodic protection in seawater, while effective, poses a real practical problem in that the current requirements change drastically with time, making it difficult to design an economical current supply system. If the initial current is sufficient to protect the structure completely from the outset, in a short time that current far exceeds the actual requirements, due to polarization and the deposition of desirable calcareous coatings of the type described in U. S. 2,200,469. On the other hand, if the initial current is of the order of that required when equilibrium is ultimately reached, months and even years may elapse before complete control of corrosion is obtained. Consequently, the designer must choose between installing a large electrical supply system, most of the capacity of which soon becomes unnecessary and represents an economic waste, and installing a minimum system, thus risking a long period of inadequate protection. The intermediate choice, that of providing a temporary source of high current in the initial stages, has not been a possible one because of the engineering difficulties and huge capital outlay involved in making portable generating equipment of the low-voltage high-current type available and transporting it from site to site.

It is therefore a principal object of the present invention to provide an improved seawater cathodic protection system which provides both the high initial current and the lower maintenance current for most effective corrosion control without occasioning economic waste. A related object is to provide a system which can be easily and inexpensively installed and which does not require a power line or rotary electrical equipment for current supply.

The invention utilizes magnesium metal anodes as the principal source of current for cathodic protection, and in essence depends for its success on the unusual electrochemical behavior of magnesium metal when operating as an anode in seawater. In this medium, mag-

2

nesium metal functioning anodically corrodes uniformly at good electrochemical efficiency and undergoes little if any polarization or coating. Extremely large currents can be generated by disposing the magnesium metal in such a shape as to have a high surface area per unit weight, and those currents can be withdrawn continuously, without significant decrease in magnitude or voltage, until the magnesium metal is almost completely exhausted. These qualities render magnesium metal uniquely suited to use in the galvanic protection of corrodible metals in seawater, and permit the design of an inexpensive, easily installed protective system.

A further discussion, by one of the present applicants, of the phenomena involved in protecting steel cathodically in seawater, and of the behavior of magnesium as an anode in that medium, has recently appeared in *Corrosion*, vol. 4, pages 358-370 (July 1948).

The protective system of the present invention essentially comprises two distinct current sources both connected to the structure to be protected so as to render it cathodic. The first or primary source, comprising high-output magnesium anodes, is a temporary one designed to provide an initial current sufficient to protect the structure at once and to polarize it completely within a few days, and then to become inoperative through exhaustion when this initial stage has been completed. The other or secondary source is a long-time one for providing continuously the smaller equilibrium current necessary to maintain the structure protected over a period of months or years. This second source also preferably comprises magnesium anodes but of relatively much lower rate of output than those of the first source.

As stated, the first current source of the system of the invention consists essentially of rapidly-expandable magnesium metal anodes submerged in the seawater and connected electrically to the structure to be protected. The shape of these anodes must be such that they provide throughout their short life an extremely high current per unit weight of magnesium. To this end, a surface area of at least 0.5 square foot per pound of magnesium metal is desirable, with areas of 0.5 to 1.3 square feet per pound being preferred. The most convenient shape consistent with this area limitation is that of a thin flexible ribbon or tape. In order to insure electrical unity during use, the ribbon should have a continuous core of metal cathodic to the magnesium metal, e. g. steel wire. In practice, a

magnesium metal ribbon having a rectangular cross-section of  $\frac{3}{8}$  inch by  $\frac{3}{4}$  inch and a core of No. 13 gauge iron wire is highly satisfactory. Such ribbon weighs 0.22 pound per foot and has a surface area of 0.85 square foot per pound. In service at the electrochemical efficiency observed in seawater, it furnishes before exhaustion slightly more than 100 ampere-hours per lineal foot.

Since the function of the primary high-surface-area anodes is to provide for the initial protection and polarization of the structure to be protected, it is essential that the mass of expendable metal be sufficient to develop the necessary quantity of electricity. To this end, the weight of ribbon or other high-area metal should correspond to at least 0.012 pound of magnesium metal per square foot of structure to be protected. However, weights much in excess of this value are unnecessary, since it is desirable for maximum economy that the high area metal be completely consumed at about the time the structure becomes fully polarized. As a practical matter, weights of 0.012 to 0.036 pound of magnesium metal per square foot of surface to be protected are ordinarily used.

With primary magnesium metal anodes of the surface area and weights just set forth, the structure to be protected receives an initial current of from 30 to 60 milliamperes per square foot for a period of about 5 to 15 days. At the end of this time, the structure will be well polarized and will have also developed a calcareous cathodic coating. The primary anodes will be almost completely expended and will cease to develop appreciable current. However, with the structure thus in equilibrium condition, it can be maintained protected by the very much smaller current provided by the secondary current source of the invention.

The equilibrium current which the secondary current source is called upon to supply is ordinarily from about 2 to 5 milliamperes per square foot of structure, depending on temperature and other factors. The source should, of course, have a capacity sufficient to supply this equilibrium current, with some reserve being desirable. Further, the source should be capable of delivering this current continuously for a period which is at least a substantial fraction of the useful life of the structure, certainly for a year or two and preferably much longer.

The secondary source may, if desired, be of the conventional generator or rectifier type. However, magnesium metal anodes are effective for this purpose also, provided they are sufficiently massive to have the necessary life and are of low surface area so that excess current is not developed. In general, slowly-expendable magnesium metal anodes should have such a shape as to have a surface area less than 0.1 square foot per pound and of such total weight as to correspond to at least 0.035 pound of magnesium metal per square foot of structure to be protected. For electrical integrity, each anode is desirably constructed with a continuous core of a metal cathodic to the magnesium metal, e. g. a steel rod or pipe. A highly satisfactory form is that of a cast cylindrical block having a diameter of 8 inches and a length of 16 inches, with a central  $\frac{3}{8}$  inch I. P. S. iron pipe core. Such an anode weighs 51 pounds, has a surface area of 0.07 square foot per pound, and, in operation in seawater, develops slightly over 3 ampere-years.

For a further explanation of the present in-

vention, reference will be made to the accompanying drawing showing the details of a preferred cathodic protection system embodying the principles already discussed. In the drawing,

5 Fig. 1 is an elevation, partly in section along the line 1—1 of Fig. 2, illustrating a steel sheet pile being protected by magnesium metal ribbon as primary current source and massive magnesium metal anodes as secondary source;

10 Fig. 2 is a reduced plan view of the installation of Fig. 1;

15 Fig. 3 is an enlarged cross-section through the magnesium metal ribbon;

15 Fig. 4 is an enlarged detailed view, in perspective, of the manner of attaching the magnesium metal ribbon to the piling; and

20 Fig. 5 is an enlarged vertical section through a massive magnesium anode, illustrating the electrical connection.

25 In the drawing, the system of the invention is being used to protect a vertical steel sheet pile bulkhead 6 immersed in seawater 7. Since the bulkhead may be of great length, only a fragment is shown. The primary current source for initially polarizing the structure is a magnesium metal ribbon 8 having a steel wire core 9. Lengths of the ribbon 8, bent into serpentine form, are attached near the top of the pile 6 above water level at spaced intervals along the bulkhead and hang 30 vertically downward into the seawater. As shown in Fig. 4, each ribbon 8 is connected firmly to the pile 6 by means of a screw-clamp 10. To insure low electrical resistance, the ribbon, clamp, and piling should all be clean and bright at the point 35 where the connection is made. The dimensions of the individual ribbons 8, and their number and spacing along the bulkhead, are chosen to provide a surface area and weight of magnesium metal within the limiting values for the rapidly-expendable primary current source already explained.

40 The secondary or long-term maintenance protective current is provided by massive cast magnesium metal anodes 11, each provided with a steel pipe core 12. As shown in Figs. 1 and 5, a group of these anodes is strung on an electrically conducting cable 13, the core of each anode being fixed mechanically and electrically to the cable by a weld 14. The cables 13 and the attached anodes are swung from eyebolts 15 mounted on steel brackets 16 welded to the pile 6 at intervals along its length. The cables are connected electrically to the brackets 16 by waterproofed low-resistance joints 17. The dimensions of the cast anodes and their number and the number and spacing of the brackets are likewise chosen to provide the surface area and weight of magnesium metal within the values for the secondary current source previously set forth.

45 While the system of the invention has been described primarily as applicable to the protection of steel in seawater, it is equally effective in protecting immersed structures of other corrodible metals no more anodic than zinc, e. g. galvanized iron and copper. The system is useful in protecting structures not only in seawater of normal salinity, but also in the diluted water found in many seaports and in the concentrated brines produced by evaporation of seawater. The term "magnesium metal" as used herein refers to magnesium and to magnesium-base alloys containing at least 85 per cent by weight of magnesium.

What is claimed is:

1. In combination with a structure immersed in seawater and formed of a corrodible metal no more anodic than zinc, a protective system of sacrificial metal submerged in the seawater near the structure and comprising a rapidly-expandable quantity of magnesium metal of such shape as to have a surface area of at least 0.5 square foot per pound and such mass as to correspond to at least 0.012 pound per square foot of structure to be protected and a slowly-expendable quantity of magnesium metal of such shape as to have a surface area less than 0.1 square foot per pound and such mass as to correspond to at least 0.035 pound per square foot of structure, all such magnesium metal being connected electrically to the structure.

2. In combination with a steel structure immersed in seawater, a protective system of sacrificial metal submerged in the seawater near the structure and comprising a rapidly-expendable quantity of magnesium metal ribbon having a surface area of at least 0.5 square foot per pound and such mass as to correspond to from 0.012 to 0.036 pound per square foot of immersed steel structure disposed close to the structure, and a slowly-expendable quantity of massive magnesium metal having a surface area less than 0.1 square foot per pound and such mass as to correspond to at least 0.035 pound per square foot of structure disposed more remotely from the structure than the ribbon, all such magnesium metal being connected electrically to the structure.

3. A system according to claim 2 wherein the magnesium metal ribbon and massive magne-

sium metal are each provided with a continuous core of metal cathodic to the magnesium metal.

4. In combination with a sheet steel structure immersed in seawater, a protective system of sacrificial metal submerged in the seawater near the structure and comprising a plurality of lengths of steel-cored magnesium metal ribbon having a surface area of at least 0.5 square foot per pound paralleling the structure, the total mass of such ribbon corresponding to from 0.012 to 0.036 pound of magnesium metal per square foot of immersed steel structure, and a plurality of massive steel-cored magnesium metal anodes each having a surface area less than 0.1 square foot per pound, the total mass of such anodes corresponding to at least 0.035 pound per square foot of structure, the said ribbons and anodes being connected electrically with the steel structure, the ribbon being so placed relative to the structure as to develop a current density at the latter of from 30 to 60 milliamperes per square foot and the massive metal being so placed as to develop at the structure a current density of from 2 to 5 milliamperes per square foot.

HAROLD A. ROBINSON.

HILARY A. HUMBLE.

#### REFERENCES CITED

The following references are of record in the 30 file of this patent:

#### UNITED STATES PATENTS

| Number    | Name        | Date          |
|-----------|-------------|---------------|
| 2,200,469 | Cox         | May 14, 1940  |
| 2,444,174 | Tarr et al. | June 29, 1948 |
| 2,478,478 | Grebe       | Aug. 9, 1949  |